

## [54] ELECTRO-OXIDATIVE METHOD FOR THE RECOVERY OF MOLYBDENUM FROM SULFIDE ORES

[75] Inventors: **Bernard J. Scheiner; Roald E. Lindstrom, both of Reno, Nev.; Thomas A. Henrie, Silver Spring, Md.**

[73] Assignee: **The United States of America as represented by the Secretary of the Interior, Washington, D.C.**

[22] Filed: **Oct. 1, 1971**

[21] Appl. No.: **185,502**

[52] U.S. Cl. .... **204/86, 204/82, 204/105 R**

[51] Int. Cl. .... **C01b 15/00**

[58] Field of Search .... **204/86, 108, 105, 94, 107, 204/82, 93**

## [56] References Cited

## UNITED STATES PATENTS

410,228 9/1889 Wiswell ..... 204/94

|           |        |                      |           |
|-----------|--------|----------------------|-----------|
| 2,761,829 | 9/1956 | Dolloff .....        | 204/112 X |
| 3,464,904 | 9/1969 | Brace .....          | 204/105 R |
| 3,639,222 | 2/1972 | Scheiner et al. .... | 204/105 R |
| 3,673,061 | 6/1972 | Kruesi .....         | 204/105 R |
| 3,755,104 | 8/1973 | Kruesi .....         | 204/94    |

## OTHER PUBLICATIONS

Khryashchev et al., Chemical Abstracts, Vol. 70, No. 4, Abstract 13618c, (p. 157), Jan. 1969.

Primary Examiner—F. C. Edmundson

Attorney, Agent, or Firm—William S. Brown; Frank A. Lukasik

## [57] ABSTRACT

This invention relates to a method for the dissolution of molybdenum and rhenium values in a sulfide-type source. These values are placed in a soluble and available form by pulverizing the source in a aqueous salt solution and electro-oxidizing it in an electrolytic cell.

5 Claims, 1 Drawing Figure





BERNARD J. SCHEINER  
 ROALD E. LINDSTROM  
 THOMAS A. HENRIE  
 INVENTOR

BY Ernest S. Cohen  
 M. Howard Silverstein  
 ATTORNEY

**ELECTRO-OXIDATIVE METHOD FOR THE  
RECOVERY OF MOLYBDENUM FROM SULFIDE  
ORES**

**BACKGROUND OF THE INVENTION**

**Field of the Invention**

This invention relates to a novel and effective method for the recovery of molybdenum and rhenium from sulfide ores, concentrates or tailings. More particularly, it relates to the dissolution of molybdenum and rhenium values in sulfide and associated source materials by an electro-oxidation process.

The major sources of molybdenum and rhenium are sulfide-type ores and the like. The classical recovery method is the use of multi-stage flotation techniques and roasting. This recovery method suffers from a number of disadvantages. Multi-stage flotation processes are relatively costly, molybdenum recovery is frequently low, and the roasting of sulfide concentrates causes heavy pollution of the atmosphere. A further disadvantage of the roasting of sulfide ores is that rhenium values are volatilized and go out the stack.

The leaching of molybdenum and rhenium values from sulfide sources has been studied by various investigators. However, in the present state of the development of the method, the reagent costs alone for hypochlorite and base makes this alternate recovery unattractive.

**THE INVENTION**

It has now been found that molybdenum and rhenium can be converted to a soluble form and extracted from their ores by an electrolytic oxidation method. In the method, an aqueous slurry of a solid sulfide-type source comprising molybdenum, rhenium, or molybdenum and rhenium, is electrolyzed while maintaining the pH of the slurry in the range 1 to 11.5, preferably 5.5 to 9. The carrier liquid for the slurry is an aqueous brine or diluted aqueous brine solution.

In the method of the invention only a nominal concentration of hypochlorite, usually less than about 0.2 weight percent, is generated. Nevertheless and surprisingly, in view of the art [see for example "Studies in Hypochlorite Leaching of Molybdenite" by R. B. Bhappu, D. H. Reynolds, and W. S. Stohmann, *Unit Processes in Hydrometallurgy*, v 24, pp. 95 - 113, Gordon & Breach Science Publishers, N.Y. (1963)] substantially quantitative solution of the molybdenum and rhenium values occurs, especially at slurry pH values in the range 5.5 to 9. Apparently the mechanism in the oxidation of the invention differs from that of the chemical hypochlorite leaching process. Applicants believe that, substantial oxidation takes place at the anode by their method.

By a solid sulfide-type source as used herein is meant by definition, molybdenum sulfide ( $MoS_2$ ) or rhenium sulfide containing ores and sulfide ores containing molybdenite or rhenium sulfide as a component, for example, copper sulfide ores and the like, flotation concentrates of sulfide ores, ore tailings and the like.

The FIGURE is a schematic flow diagram illustrating a particular mode of the invention, utilizing a bipolar flow-through cell for the electro-oxidative dissolution of the molybdenum present in a sulfide ore.

**EMBODIMENT**

In a preferred embodiment of the invention as illustrated in the flow diagram of FIG. 1, a process unit 5 comprising a bipolar cell, 3, and a stirred surge and agitation tank 7 are joined by suitable transfer lines 4, 8, 9 and 2 and the unit is used in the electro-oxidation of an aqueous slurry (pulp) of a typical low-grade molybdenite ore, for example an ore containing about 0.2 10 weight percent of molybdenum sulfide, minor amounts of copper sulfide, iron sulfide and sulfur and having as the major components quartz and potassium feldspar. Via lines 1, 2 and 1, 8, 9, a slurry of the ore is charged to the cell 3, and the surge tank, 7. The liquid component of the slurry is an aqueous brine solution containing about 10 weight percent chloride. The solid component of the slurry is the above described ore which has been pulverized to below 35 mesh (U.S. Standard Mesh) with about 65 percent of the solid being below 15 200 mesh. Each 100 parts by weight of the slurry desirably contain about 10 parts of the pulverized ore.

During the electro-oxidation, by means of suitable pumps not shown, the slurry is circulated as indicated, including introduction of the circulative slurry into the cell at the base, via lines 9, 8 and 2, thence up through the bipolar (graphite) electrodes and then withdrawal from the cell via line 4 for delivery to the stirred surge tank 7.

For the electro-oxidation, the following conditions 30 are employed:

|                                                      |         |
|------------------------------------------------------|---------|
| Current density, amps/ sq. inch                      | 0.5     |
| Power consumption, kw/hrs/lb of Molybdenum Extracted | 25      |
| Slurry pH                                            | 5.5-6/5 |
| Slurry Temp, °C                                      | 30-60   |
| Time, Average slurry residence time in cell, hours   | 3.5     |

with the pH being maintained by the addition via line 40 5 of solid sodium carbonate ( $Na_2CO_3 \cdot H_2O$ ) as required (total consumption rate of 5 lbs. per lb. of Molybdenum dissolved).

Under the above conditions 95 plus percent of the molybdenum sulfide values in the ore are converted to the soluble salt, sodium molybdate. Where the ore contains a rhenium sulfide component, it too is dissolved in the form of the sodium perrhenate salt. Via line 10, the electro-oxidized slurry is withdrawn from the cell-surge tank unit and is passed to a suitable liquid-solid separator, 11, for example a settling tank or a filter unit and separated. The depleted ore tails are discharged from the system by a suitable means, for example a wash-out line 13.

The pregnant electro-oxidation brine containing the dissolved molybdenum as sodium molybdate, is withdrawn from the separator means, 11, and is passed to a suitably molybdate recovery unit, for example an ion exchange unit 19, via line 15, [see for example; (1) *Ion Exchange Technology* by G. Nachad and J. Schubert, Academic Press, N.Y., 1956; (2) *Modern Methods for the Separation of Rarer Metal Ions*, (p 506) by Korkisch, J., Pergamon Press (1969); (3) *Anal Chem*, (v. 36, p 1654) (1964) by Hamaguchi, H., Kawabuchi, K., and Kuroda, R.; and (4) *J. of Chromatography*, (v 17, p 567) (1965) by Hamaguchi, H., Kawabuchi, K., and Kuroda, R.; or a liquid-liquid extraction, see for example *Zeitschrift Chemi* (v 8, p 235 (1968) by Fisher, C.,

Muhl, P. and Gunzler, G.J. The brine, essentially stripped of its molybdenum content, is withdrawn from the ion exchange unit, 19, via line 21, and is desirably recycled to the process together with make-up brine as required to satisfy the concentration and volume conditions described above for the process. The molybdenum values may be recovered via line 16.

The preparation of the slurry is by ordinary means, including the grinding of the ore or feed material, and usually is carried out in the presence of the brine carrier liquid. The solid-liquid content of the slurry is adjusted as desired, and the slurry is passed to the process as described above.

#### VARIABLE

Depending upon the particular molybdenum sulfide-type feed source, the operational requirements for a satisfactory electro-oxidation process may vary somewhat. In general, however, the process parameters are as follows:

##### A Brine (electrolyte), Concentration and Kind

The concentration of the electrolyte (salt) may vary from a minor amount, for example 0.1 weight percent up to the saturation value. Best results are, in general, experienced when the concentration is in about the 7 to 20, preferably 9 to 15 weight percent range. The use of brine concentrations above about 15 weight percent and below about 7 percent is relatively inefficient.

Alkali metal, ammonium and alkaline earth metal salts, especially the chlorides (water soluble substantially ionized salts), and mixtures of these salts are satisfactory electrolytes for use in the process. Sodium chloride is preferred for a number of reasons including low cost.

##### B The Slurry

The particle sizing and solids content of the slurry may vary over a substantial range. In general a useful dissolution of molybdenum sulfide values in a pulverized solid feed is experienced when the particles are sized to pass through a 35 mesh screen. The comparative examples 1 - 4 in Table 1 following, demonstrate, however, that better results are to be expected when at least about 50 percent of the solid particles passes through a 200 mesh screen. These examples were carried out in a glass cell fitted for stirring and using graphite electrodes as follows:

#### Conditions:

|  |     | Temp. °C 30                               |
|--|-----|-------------------------------------------|
|  | 0.5 | Current Density,<br>Amperes per. sq. inch |
|  | 4   | Treatment<br>Amperes                      |
|  | 8   | Time, hours                               |

TABLE 1

| 10 | Ex no | Particle Size<br>% — 200 mesh | Molybdenum<br>% dissolved |
|----|-------|-------------------------------|---------------------------|
|    | 1     | 36                            | 73                        |
|    | 2     | 48                            | 86                        |
|    | 3     | 61                            | 90                        |
| 15 | 4     | 68                            | 94                        |

##### B. (forward)

The solid content of the slurry may vary over a wide range. The slurry must be pumpable. For practical purposes at least about 1 part of solid per 100 parts of slurry should be present. In general, good results are obtained when the solid content of the slurry is in the range 1 to 60 parts per 100 parts (weight). A solid content of 1 to 15 parts to 100 parts solution is preferred when treating higher grade ores or concentrates, whereas a solid content of 30 to 40 parts to 100 parts solution is preferred when treating low grade ores.

##### C. Slurry pH

Molybdenum pH, i.e., values can be electro-oxidized over a large range of pH, i.e., from about 1 to 11.5. Excellent results are in general experienced when the slurry pH is maintained in the range 5 to 9, preferably 5.5. to 6.5. Sulfuric acid is a by-product of the oxidation; therefore in order to maintain the pH, a suitable inorganic base must be added during the course of the oxidative extraction of the molybdenum. Alkali metal and ammonium carbonates and hydroxide and the like are useful for this purpose. A solid such as  $\text{Na}_2\text{CO}_3\text{H}_2\text{O}$  is especially desirable since the addition in the solid form results in no appreciable dilution of the slurry. The contrary is the case where the addition is by the use of an aqueous solution of a suitable base.

The effect of the amount of the base added and the resulting pH is illustrated in examples 5 - 8 below which were carried out as in example 1 except that the amount of base added was varied as noted in Table 2 with the results as follows:

TABLE 2

| Ex.<br>No. | $\text{Na}_2\text{CO}_3\text{H}_2\text{O}$<br>grams | Tails<br>%Mo | Mo Extracted,<br>% | pH   | Base Consumption<br>lb Na CO <sub>3</sub> /lb Mo<br>ext'd |
|------------|-----------------------------------------------------|--------------|--------------------|------|-----------------------------------------------------------|
| 5          | 16                                                  | 0.01         | 95.2               | 13.7 | 7.18                                                      |
| 6          | 13                                                  | 0.01         | 95.2               | 11.1 | 5.38                                                      |
| 7          | 10                                                  | 0.01         | 95.2               | 8.5  | 4.46                                                      |
| 8          | 8                                                   | 0.015        | 92.9               | 6.85 | 3.59                                                      |

#### Charge

|                          |                               |
|--------------------------|-------------------------------|
| Solid Feed               | Pulverized ore or concentrate |
| Sizing                   | MoS <sub>2</sub>              |
| Electrolyte              | Below 35 Mesh                 |
|                          | Aqueous sodium chloride       |
| Salt Concentration, wt % | 10                            |
| Slurry, grams            | 90                            |
| Salt solution, wt. %     | 10                            |
| Solid Feed, wt. %        | 10                            |
| Base                     | $\text{Na}_2\text{CO}_3$      |
| Amount, gr               | 16                            |

#### EXAMPLE 9

Example 7 was repeated except that the slurry was sampled during the course of the electro-oxidation after 2, 3, 3.5 and 4 hours of extraction time had elapsed and the samples were analyzed with the following result:

| Time | % Mo Extracted |
|------|----------------|
| 2    | 58             |
| 3    | 85             |

| Time | % Mo Extracted |
|------|----------------|
| 3.5  | 95             |
| 4    | 95             |

This example demonstrated that the extraction was essentially complete after a residence time of 3.5 hours. At this time the power consumption was 24.5 kilowatt hours per pound of molybdenum extracted.

#### D. Temperature

The effect of temperature upon the electro-oxidation is demonstrated in the examples 10 – 13 of Table 3 below. These were carried out as in examples 1 – 4 except that the temperature was varied as indicated.

TABLE 3

| Ex. No. | Temp., °C | Tails, wt. % Molybdenum | Extraction % |
|---------|-----------|-------------------------|--------------|
| 10      | 30        | 0.01                    | 95.2         |
| 11      | 40        | 0.01                    | 95.2         |
| 12      | 50        | 0.01                    | 95.2         |
| 13      | 60        | 0.25                    | 88.1         |

These data demonstrate that the slurry temperature may vary over a range, i.e., from above the freezing point and below the boiling point of the aqueous brine. Preferably the slurry temperature should be in the range below about 55°C and above about 15°C. In the processing of a low-grade ore, temperature control may be effected easily by one or more ordinary electrolysis parameters, including variations in salt concentration, pulp density, current density, size and shape of the cell and the surge tank, and electrode spacing. However, when a molybdenum sulfide concentrate is employed, conventional means such as indirect heat exchangers, cooling towers and the like are desirably used to maintain the slurry temperature below about 55°C.

#### E. Treatment Rate, Ampere-hours

The treatment rate desirably used, varies depending upon the characteristics of the particular ore and slurry being employed. The effect of the rate in the case of the representative low-grade ore described above is demonstrated in examples 14 – 16 of Table 4 which were carried out as in Example 1 except at different rates as indicated.

TABLE 4

| Ex. No. | Amperes (1) | Treatment Time, Hrs. | Tails, wt. % Mo | Mo Extracting % |
|---------|-------------|----------------------|-----------------|-----------------|
| 14      | 4           | 8                    | 0.10            | 95.2            |
| 15      | 8           | 4                    | 0.10            | 95.2            |
| 16      | 16          | 2                    | 0.03            | 85.8            |

(1) Current density 0.5 amperes/inch<sup>2</sup>.

Examples 14 – 16 show that for a given slurry there is an optimum treatment rate which when exceeded results in a less efficient utilization of power. However, a wide range of treatment rates can be employed and yet result in a satisfactory molybdenum dissolution and recovery. The rate desirably used for a particular slurry is readily determinable by routine tests, for example as illustrated in examples 9 – 11.

#### F. Current Density

The current density, amperes per square inch of electrode, may vary over a range. The use of a current density in the range 0.1 to about 2 amperes per square

inch, in general, effects a useful dissolution. However, as illustrated in the examples 17 – 19 of Table 5 (carried out as Example 1 except with the current density as noted), for a given slurry, electrode spacing and the like, there is an optimum current density (as related to power utilization, cell sizing and capital costs).

TABLE 5

| Ex. No. | Current Density Amps/inch <sup>2</sup> | Molybdenum extracted, % |
|---------|----------------------------------------|-------------------------|
| 17      | 0.5                                    | 95.2                    |
| 18      | 1.0                                    | 65.3                    |
| 19      | 1.5                                    | 65.3                    |

In general, the employment of a current density in the range 0.2 to 1.0 amperes per square inch is most effective and of this range, the use of about 0.5 ampere per square inch is preferred.

#### G. The Cell

The electrolysis unit requirements of the method of the invention may be satisfied by use of a standard cell arrangement and should include sufficient agitation to prevent settling of the particulate solid component of the slurry. The bipolar flow through the type cell as illustrated in the FIGURE is preferred. However, an ordinary plate cell is often advantageously employed, especially for the electro-oxidation of a low grade ore.

Graphite electrodes are in general most satisfactory for use in the method. Other materials of construction such as copper, iron and the like are also suitable for use in fabricating the cathode. Anodes constructed of PbO<sub>2</sub> or RuO<sub>2</sub> coated materials and the like are also suitable.

The spacing between the electrodes may vary somewhat depending upon the particle sizing of the solid, the concentration of the electrolyte and the like. In general a spacing of about one-half inch is satisfactory.

#### H. Time

The time required to achieve a satisfactory recovery of the molybdenum and rhenium values in a solid feed varies depending upon the degree of recovery desired, the brine concentration, the current density used and the like variables. In general a useful recovery can be effected in a process in which the average residence time of the slurry in the cell (electrode portion) is in the range 1 to 20 hours. In general, best results, in terms of economic factors, obtain from the use of average residence times in the range 2.5 to 5 hours.

The foregoing examples were carried out using molybdenum sulfide-type feeds. Essentially the same results are experienced when the feed contains a rhenium sulfide-type component or a mixture of molybdenum and rhenium sulfide materials. Like molybdenum, the rhenium values are conveniently recovered by the use of known ion exchange extraction beds (resins) and techniques (see above listed references). In the case of rhenium, the oxidized form is the sodium (or ammonium, etc.) perrhenate. These examples and the disclosure demonstrate that the method of the invention is a useful effective means for the dissolution of molybdenum and rhenium from sulfide-type solids, ores, tailings or the like, rendering them to a form (i.e., as solutes) from which a facile recovery by ordinary means can be made.

Those of skill in the art in view of the examples and disclosure herein will appreciate that numerous varia-

tions in the conditions and feeds and combinations thereof may be made and yet these variations remain within the scope of the claimed invention.

We claim:

1. The method for the dissolution of molybdenum and rhenium, which comprises:  
forming a pumpable slurry, said slurry being a mixture of a pulverized solid and a carrier liquid, said solid being a sulfide-type source of molybdenum, or rhenium or of molybdenum and rhenium; and said carrier liquid being an aqueous salt solution; contacting said slurry with an anode and cathode; providing current through said anode and cathode, while maintaining the slurry at a pH of 5 to 9 and temperature of 15° to 55°C, and thereby electrolyzing said slurry to electro-oxidize said molybdenum and rhenium; and

separating the resulting slurry into two fractions the first of which is an aqueous solution containing dissolved molybdenum, rhenium or a mixture of dissolved molybdenum and rhenium, and the second of which is the depleted electrolyzed solid.

2. The method as in claim 1 where said electrolysis is carried out in a bipolar flow-through cell containing graphite electrodes or in a stirred plate cell.

3. The method as in claim 1 wherein said dissolved molybdenum is removed by an extraction method and the resulting aqueous salt solution is recycled for use in forming a subsequent slurry.

4. The method of claim 1 in which the temperature of the slurry is maintained at about 30° to 50°C.

5. The method of claim 1 in which the pH of the slurry is maintained at about 5.5 to 6.5.

\* \* \* \* \*

20

25

30

35

40

45

50

55

60

65